# EUROPEAN PATENT SPECIFICATION

(11) **EP 0 649 914 B1**
(45) Date of publication and mention of the grant of the patent: **04.03.1998**
(21) Application number: 94401992.6
(22) Date of filing: 07.09.1994
(51) Int. Cl.: C22C 38/04, C21D 6/00, C21D 8/00

(54) **An Fe-Mn vibration damping alloy steel and a method for making the same**
Fe-Mn Stahl mit guten Schwingungsdämpfungseigenschaften und Verfahren zu dessen Herstellung
Acier de type Fe-Mn présentant d'excellentes propriétés d'amortissement de vibrations et procédure pour sa fabrication

(30) Priority: 22.10.1993 KR 9321973
(43) Date of publication of application: 26.04.1995
(73) Proprietor: WOOJIN OSK CORPORATION, Youngin-gun, Kyoungki-do (KR)
(72) Inventor: Choi, Chong-Sool, Mapo-ku, Seoul (KR); Jun, Joong-Hwan, Kangnam-ku, Seoul (KR); Ko, Young-Sam, Dobong-ku, Seoul (KR); Lee, Man-Eob, Kwachun-si, Kyungki-do (KR); Baek, Seung-Han, Sungnam-si, Kyungki-do (KR); Son, Yong-Chul, Sungnam-si, Kyungki-do (KR); Kim, Jeong-Cheol, Seoul (KR)
(74) Representative: Keib, Gérard

(56) References cited:
- WO-A-90/00629
- TAEHAN KUMSOK HAKHOECHI, vol. 32, no. 2, 1994 DEP. METALL. ENG., YONSEI UNIV., SEOUL, KOREA, pages 240-245, HAN, J.S., PARK, H.R., CHOI, C.S. 'Stress Induced Martensitic Transformation Behaviour of Fe-17Mn Alloy '
- METALL. TRANS. A, vol. 18A, no. 6, 1987 FAC. ENG., IBARAKI UNIV., HITACHI, JP, pages 1073-81, TOMOTA, Y., STRUM, M., MORRIS, J. 'The Relationship Between Toughness and Microstructure in Iron-High Manganese Binary Alloys'
- KRIST. TECH., vol. 11, no. 6, 1976 WISSENSCHAFTSBER. WERKSTOFFKD., WILHELM-PIECK-UNIV., ROSTOCK, DDR, pages 663-671, SCHUMANN, H. 'Crystallography of Martensitic epsilon alpha Lattice Transformation'
- PATENT ABSTRACTS OF JAPAN vol. 18 no. 30 (C-1153) ,17 January 1994 & JP-A-05 255813 (NIPPON STEEL CORP.) 5 October 1993,
- POROSHK. METALL. (KIEV), vol. 12, 1986 NPO'TULACHERMET', USSR, pages 52-55, BYCHIKHIN, G.A., GONCHARENKO, I.A., IL'IN, A.N., KALLISTRATOV, D.N., MARKOVA, G.V., SKURIKHIN, M.N. 'Effect of epsilon Phase Content on the Vibration Damping Properties of Powder Metallurgy Iron-Manganese Alloy '
- MATER. TRANS., JIM , vol. 34, no. 6, 1993 FAC. ENG., KYUSHU UNIV. FUKUOKA, 812, JP, pages 489-495, TAKAKI ET AL 'Effects of Austenite Grain Size on epsilon Martensitic Transformation in Fe-15%Mn Alloy'

## Description

### BACKGROUND OF THE INVENTION

### (1) Field of the Invention

The present invention relates to a method for making an Fe-Mn vibration damping alloy steel at a low production cost.

### (2) Description of the Prior Art

In line with a trend for high-grade and high precision aircraft, ships, automotive vehicles and various machinery, vibration damping alloy is widely used in the many kinds of machine parts that are sources of vibration and noise. Study of vibration damping alloys has been lively because of the increase in demand for such alloys.

Vibration damping alloys developed and used so far are classified into following types: Fe-C-Si and Al-Zn which are of the composite type; Fe-Cr, Fe-Cr-Al and Co-Ni which are of the ferromagnetic type; Mg-Zr, Mg and Mg₂Ni which are of the dislocation type;- and Mn-Cu, Cu-Al-Ni and Ni-Ti which are of the twin type. The above vibration damping alloys have excellent vibration damping capacities but have poor mechanical properties. Thus, the alloys cannot be used widely; and since they contain a lot of expensive elements, the production costs are high, limiting the industrial use of the alloys.

A solution of the above problem is disclosed in U.S. Patent No. 5,290,372 (Jong-Sool Choi, et al.) and in an article of Metallurgical Transactions A, Vol. 18A, June 1987, titled 'The relationship between toughness and microstructure in Fe high Mn binary alloys', by Tomota, Strum and Morris. These two disclosures describe Fe-Mn (10 to 22%) and (16-36% respectively) vibration damping alloy steels having a partial martensitic structure. As a method for making the alloy, an Fe-Mn (10-22%) ingot is homogenized at 1000°C to 1300°C for 20 to 40 hours and hot-rolled. After solid solution treatment of the ingot at 900 to 1100°C for 30 minutes to an hour, air cooling or water quenching is carried out to produce a partial epsilon martensite from the parent phase, austenite. This damping mechanism is entirely different from those of the conventional damping alloys, and has a characteristic of absorbing vibrational energy by movement of the ε/γ interface under external vibration stress. However, we have made an effort to further improve excellent vibration damping alloy steels and we succeeded in inventing a vibration damping alloy steel of the present invention.

### SUMMARY OF THE INVENTION

The method of the present invention is given in the single claim.

### BRIEF DESCRIPTION OF THE DRAWINGS

FIG. 1 is a binary phase diagram of an Fe-Mn alloy;
FIG. 2 shows a transformation amount of the Fe-Mn alloy at room temperature;
FIG. 3 shows specific damping capacities according to the amount of cold rolling of the Fe-17%Mn alloy; and
FIGS. 4A to 4D show free vibration damping curves before and after cold rolling of a comparative alloy and an alloy of the present invention, specifically,
FIG. 4A shows a free vibration damping curve before cold rolling an Fe-4%Mn alloy (as water-quenched);
FIG. 4B shows a free vibration damping curve after cold rolling the Fe-4%Mn alloy;
FIG. 4C shows a free vibration damping curve before cold rolling Fe-17%Mn alloy (as water-quenched) ; and
FIG. 4D shows a free vibration damping curve after cold rolling the Fe-17%Mn alloy.

### DETAILED DESCRIPTION OF THE PRESENT INVENTION

In making the alloy steels according to the present invention, an amount of electrolytic iron and an electrolytic manganese is weighed to contain 10 to 24% manganese by weight and the remainder iron. The iron is melted first by heating in a melting furnace at more than 1500°C; and then the manganese is charged and melted.

After that, the melted mixture is cast into a mold to produce an ingot. Subsequently, the cast ingot is homogenized at 1000°C to 1300°C for 12 to 40 hours and then the homogenized ingot is hot-rolled to produce a rolled metal of a predetermined dimension.

The rolled metal is subjected to a solid solution treatment at 900°C to 1100°C for 30 to 60 minutes and cooled by air or water. Finally the rolled metal is again cold rolled around room temperature (25°C ± 50°C) so as to have a reduction rate of 5-25%, thereby obtaining Fe-Mn alloy steels having high vibration damping capacities.

The reason why the above condition is determined in the present invention is as follows. The homogenizing condition is defined to be at 1000°C to 1300°C for 12 to 40 hours so that the manganese, the main element, may be segregated during the period of time the ingot is cast. Thus, when the ingot is heated at a high temperature of 1000°C to 1300°C, the high concentrated manganese is diffused into a low concentration region which homogenizes the composition of the manganese.

If homogenization of the ingot is performed at temperatures below 1000°C, the diffusion rate becomes slower. Therefore it takes more then 40 hours to homogenize, and the production cost is increased. If the temperature for the homogenization is more than 1300°C, the homogenization time may be reduced to be within 12 hours, but a local melting phenomenon may occur at the grain boundary where the manganese is segregated during casting. Accordingly, the homogenization is preferably performed at 1000°C to 1300°C for 12 to 40 hours.

The solid solution treatment is performed at 900°C to 1100°C for 30 to 60 minutes. If the treatment is carried out at higher than 1100°C, the grains of the alloys are coarsened which deteriorates the tensile strength. If the temperature is too low, such as less than 900°C, the grains become so small that raising the tensile strength decreases the martensite start temperature(Ms). Thus, a small amount of epsilon martensite is produced and the damping capacity is lowered. Accordingly, the optimum condition to have both excellent tensile strength and damping capacity is at 900°C to 1100°C for 30 to 60 minutes.

The alloy of the present invention contains manganese of 10 to 24% by weight, see, FIG. 1 of the binary phase diagram. The alloys which contain up to 10% manganese create α' martensite, the alloys which contain from 10 to 15% manganese create a 3-phase mixture structure of ε + α' + γ, and the alloys which contain from 15 to 28% manganese create a 2-phase mixture structure of ε+γ.

The Fe-Mn vibration damping mechanism, as mentioned above, absorbs vibration energy by movement of the ε/γ interface under external vibration stress. If the manganese alloy is less than 10% Mn only one phase, α' martensite is created and the vibration damping effect hardly occurs. Since ε and γ martensites are extensive in the 10 to 28% Mn alloys, a lot of ε/γ interfaces exist which yields high vibration damping effects.

However, if cold rolling is carried out in the alloy of these compositions at around room temperature (25°C±50°C), more martensite is induced by the external stress which increases the total interfacial area of the ε/γ interface. Thus, the damping capacity is remarkably more enhanced than before cold rolling. If, however, the amount of Mn is more than 24%, the Neel temperature of austenite, Tn (i.e., a magnetic transition temperature at which paramagnetic is changed to antiferromagnetic), is higher than the room temperature, and the austenite is stabilized. Therefore, greater amounts of cold rolling at around room temperature can produce the ε martensite, and simultaneously, the slip system of the austenite operates to generate a great density of dislocations. Since these dislocations act as an obstacle against the movement of the ε/γ interface during vibrations, the damping capacity cannot be improved by cold rolling when the alloy has more than 24% Mn by weight. Accordingly, the composition of Mn is defined to the range of 10 to 24% because ε martensite is produced preferentially by cold rolling at around room temperature without slip dislocation.

If the cold rolling is performed at a reduction of less than 30% at around the room temperature, more fine and thin ε plates are produced inside by the cold rolling which increases the total interface area of the ε/γ interface, and higher vibration damping capacity is obtained than before the cold rolling. If the amount of cold rolling is increased to more than 30%, coalescence of ε martensite plates occurs, and hence the ε/γ interface area is reduced. The martensite produced in this way restrains the movement of the ε/γ interface, and a lot of dislocations are produced inside the ε and γ martensites which interact with the ε/γ interface disturbing the movement of the ε/γ interface and thereby degrading the vibration damping capacity.

The alloy of the present invention may contain carbon of up to 0.2% by weight, silicon of up to 0.4% by weight, sulfur of up to 0.05% by weight, and phosphorus of up to 0.05% by weight as impurities.

If the amount of impurities is higher, the impurity elements are diffused to the ε/γ interfaces which locks the interface, and movement of the ε/γ interfaces is difficult, thereby degrading the vibration damping capacities.

Table 1 shows the comparison of results of the vibration damping capacities in the alloy of the present invention and the conventional alloy according to the cold rolling process.

The alloy of the present invention that has undergone cold rolling has a superior vibration damping effect compared to the alloy that is not cold rolled.

**TABLE 1**

| Name of Alloy | Specific Damping Capacity (SDC) | | | | | | Note |
|---|---|---|---|---|---|---|---|
| | | Air-Cooled | Water-Quenched | 10% Cold-Rolled | 20% Cold-Rolled | 35% Cold-Rolled | |
| Fe-8% | Mn | 6 | 6 | 6 | 6 | 5 | Comparative Alloy steel |
| Fe-10% | Mn | 10 | 10 | 14 | 14 | 9 | Alloy steel with composition according to the present invention |
| Fe-13% | Mn | 12 | 12 | 16 | 16 | 11 | |
| Fe-15% | Mn | 15 | 15 | 20 | 20 | 14 | |
| Fe-17% | Mn | 25 | 25 | 30 | 30 | 23 | |
| Fe-20% | Mn | 25 | 25 | 30 | 30 | 23 | |
| Fe-23% | Mn | 22 | 22 | 27 | 27 | 21 | |
| Fe-24% | Mn | 15 | 15 | 20 | 20 | 14 | |
| Fe-26% | Mn | 9 | 9 | 10 | 10 | 9 | Comparative Alloy steel |
| Fe-4% | Mn | 5 | 5 | 5 | 5 | 5 | Comparative Alloy steel |
| Carbon Steel | | 5 | 5 | 5 | 5 | 5 | Conventional Steel |

FIG. 1 shows the Fe-rich side of Fe-Mn binary phase diagram which is the basis of this invention. Transformation temperatures of each phase are determined using a dilatometer by cooling at a rate of 3°C/min. In FIG 1, α' martensite is formed in the case of up to 10% Mn by weight. There is a mixture structure of ε + α' + γ in the case of 10 to 15% Mn by weight. There is a dual phase structure of ε + γ in the case of 15 to 28% Mn by weight and a single phase structure of γ in the case of more than 28% Mn by weight.

FIG. 2 shows a volume fraction of each phase by an X-ray diffraction analysis method after each alloy is subjected to solid solution treatment at 1000°C and air-cooled to the room temperature.

As shown in Tables 1 and 2 and FIGS. 1 and 2, the Mn percentages by weight corresponding to α' martensitic alloy have a poor vibration damping capacity and the alloy of ε + α' + γ mixture structure has excellent vibration damping capacity as well as tensile strength.

Table 2 shows a comparison of vibration damping capacities according to martensitic structure in case of 10% reduction by cold rolling.

**TABLE 2**

| Name of Alloy | Structure | Specific Damping Capacity (SDC) | Tensile Strength (Kg/mm2) |
|---|---|---|---|
| Fe - 4% Mn | α' martensite | 5 | 66 |
| Fe - 17% Mn | ε+α'+γ martensite | 30 | 70 |
| Low Carbon Steel | Tempered martensite | 5 | 49 |

The alloy having the ε + α' + γ mixture structure has a greater vibration damping capacity than that of α' martensitic alloy, because the sub-structure of the α' martensite consists of dislocations and absorbs vibration energy by movement of the dislocations. In the alloy of the ε + α' + γ mixture structure, if the alloy receives vibrational stress, the ε/γ interface moves and absorbs vibration energy yielding an excellent vibration damping capacity.

FIG. 3 shows the variation of a specific damping capacities according to the amount of cold rolling in case of the Fe-17% Mn alloy. The specific damping capacity (SDC) is increased in accordance with the increase in the amount of cold rolling, and maximum vibration damping capacity is presented at the reduction rate from 10 to 20%. If the amount of cold rolling is more than about 20%, the SDC is decreased. If the amount of cold rolling is more than about 30%, the vibration damping capacity is less than the vibration damping capacity without cold rolling. The method according to the present invention stipulates 5-25% cold rolling reduction rate.

FIGS. 4A to 4D show free vibration damping curves of a comparative alloy and the alloy of this invention before and after the cold rolling. These curves were measured by means of a torsional pendulum type measuring apparatus at the maximum surface shear strain of γ = 8 x 10⁻⁴, using a round shape specimen. The comparative alloy (Fe-4%Mn) has a small vibration damping capacity after water quenching (FIG. 4A), and the vibration damping effect is not improved even with 15% reduction by cold rolling (FIG. 4B). However, as an example of one alloy of this invention, Fe-17%Mn alloy has a remarkable vibrational amplitude decay after water quenching for high temperature rolling (FIG. 4C). However, if 15% reduction by cold rolling is further carried out at the room temperature, the vibrational amplitude decay is more remarkable as shown in FIG. 4D.

The alloys of this invention, as mentioned above, have vibration damping capacities and mechanical properties which are superior to conventional alloys.

While this invention has been described in connection with what is presently considered to be the most practical and preferred embodiments, it is to be understood that the invention is not limited to the disclosed embodiments, but, is intended to cover various modifications and equivalent arrangements included within the scope of the appended claim.

## Claims

1. A method for making an Fe-Mn vibration damping alloy steel, comprising the steps of:
melting an alloy consisting of 10 to 24 % manganese by weight, remaining iron and unavoidable impurities to produce a melted alloy ;
casting the melted alloy into a mold to produce a metal ingot ;
heating the ingot at a temperature of 1000°C to 1300°C for 12 to 40 hours to homogenize the ingot, and hot-rolling the homogenized ingot to produce a rolled alloy steel;
performing a solid solution treatment on the alloy steel at 900 to 1100°C for 30 to 60 minutes ; and
cooling the alloy steel by air or water to room temperature ;
characterized by further comprising, cold rolling the alloy steel at a reduction rate of 5 to 25 % around room temperature.

## Patentansprüche

1. Verfahren zur Herstellung von Fe-Mn vibrationsdämpfenden Stahllegierungen, enthaltend die Schritte:
- Aufschmelzen einer Legierung enthaltend 10 bis 24 Gewichtsprozent Mangan, verbleibender Anteil Eisen und unvermeidbare Verunreinigungen zum Herstellen einer geschmolzenen Legierung;
- Gießen der geschmolzenen Legierungen in eine Form zum Herstellen eines metallischen Blockes;
- Erhitzen des Blockes auf eine Temperatur von 1000°C bis 1300°C über 12 bis 40 Stunden zum homogenisieren des Blockes, und Warmwalzen des homogenisierten Blockes zur Herstellung einer gewalzten Stahllegierung;
- Durchführen einer Behandlung in fester Lösung mit der Stahllegierung bei 900 °C bis 1000°C über 30 bis 60 Minuten, und
- Abkühlen der Stahllegierung durch Luft oder Wasser auf Raumtemperatur;
**gekennzeichnet durch darüber hinaus aufweisend**
- Kaltwalzen der Stahllegierung mit einer Reduktionsrate von 5-25% ungefähr bei Raumtemperatur.

## Revendications

1. Procédé pour fabriquer un acier en alliage amortissant les vibrations à base de Fe-Mn, comprenant les étapes consistant à:
faire fondre un alliage constitué de 10 à 24% en poids de manganèse, le reste étant du fer et des impuretés inévitables, pour produire un alliage fondu;
couler l'alliage fondu dans un moule pour produire un lingot métallique;
chauffer le lingot à une température de 1 000°C à 1 300°C pendant 12 à 40 heures pour homogénéiser le lingot, et laminer à chaud le lingot homogénéisé pour produire un acier d'alliage laminé;
réaliser un traitement en solution solide sur l'acier d'alliage, à une température de 900 à 1 100°C pendant 30 à 60 minutes; et
refroidir l'acier d'alliage à l'air ou à l'eau à la température ambiante;
caractérisé en ce qu'il consiste, en outre, à laminer à froid l'acier d'alliage à un taux de réduction de 5 à 25% aux alentours de la température ambiante.
